

No. 811,017.

PATENTED JAN. 30, 1906.

O. WIEDERHOLD.  
PROCESS OF MAKING MANTLES.  
APPLICATION FILED MAR. 6, 1905.

FIG. 1.

UNBLEACHED KNITTED TUBE



FIG. 2.

BLEACHED



FIG. 3.

IMPREGNATED



WITNESSES:

Joe Whiting  
Rene Meune

INVENTOR:

Oscar Wiederhold,

By Attorneys,

Arthur C. Fraser & Co.

# UNITED STATES PATENT OFFICE.

OSCAR WIEDERHOLD, OF JERSEY CITY, NEW JERSEY.

## PROCESS OF MAKING MANTLES.

No. 811,017.

Specification of Letters Patent.

Patented Jan. 30, 1906.

Application filed March 6, 1905. Serial No. 248,680.

*To all whom it may concern:*

Be it known that I, OSCAR WIEDERHOLD, a citizen of the United States, residing in Jersey City, in the county of Hudson and State 5 of New Jersey, have invented certain new and useful Improvements in Processes of Making Mantles, of which the following is a specification.

Mantles for incandescent gas-burners are 10 made by knitting or otherwise working cotton or other textile material into the desired form and impregnating the same with the refractory material which becomes incandescent under the heat of the flame of the burner. 15 The refractory materials whose incandescence produces the light are usually thorium and cerium. The photometric value of the mantle depends largely on the purity of the incandescent substance or substances. Considerable 20 reduction of efficiency is occasioned by the presence of iron or other impurities.

The object of this invention is to provide a process of making the mantles which shall eliminate to a greater extent than has been 25 possible by previous processes impurities which reduce the efficiency of the mantle. At the same time the improved process is cheaper than processes heretofore used in the manufacture of good mantles. It is generally understood 30 that at least a considerable percentage of the iron or other impurities in the mantles is present in the cotton, in which it is taken up in minute quantities from the soil. It has been customary, therefore, to bleach the crude

35 spun cotton, first boiling it in an alkaline solution in order to remove the oily substances and facilitate the bleaching operation. It was then bleached in loose skeins in chlorid of lime or any one of various other well-known

40 bleaching agents after which it was spooled, and then knitted into the usually tubular form of the mantle. In the spooling and knitting machines it is found that the cotton receives further impurities by way of minute quantities of iron from the needles and dirt from 45 the oils of the machines. It has been necessary, therefore, to wash the knitted material in acid followed by an ammonia solution or by boiling in distilled water or in other ways

50 to remove these impurities before the material was dried and dipped in or otherwise impregnated with the usual solution of nitrate of thorium and cerium.

According to this invention a great improvement 55 is effected by first knitting or otherwise forming the crude cotton or other tex-

tile material into the desired shape and subsequently bleaching it.

An example of the process in detail is as follows: The crude spun cotton is knitted into 60 the desired form, washed in alkali to remove the oily matters, and bleached. It is then thoroughly washed to bodily remove the impurities, which were oxidized but not removed by the bleaching operation, after which it is 65 dried and impregnated with the incandescing material. The new process eliminates to a marked degree impurities which seriously interfere with the light-giving power of mantles made by the old process. For example, 70 other considerations being exactly the same, I have found that the number of "seconds"—that is, mantles below the commercial standard—were from eight per cent. to twenty per cent. when made by the old process and are 75 only from one-half to one per cent. when made by the new process, using the same photometric standard. Furthermore, the mantles made by the new process are of much more uniform quality than those made by the old 80 process.

Irregularities in the product have heretofore been very wide even where the manufacture has been conducted with great care, and this irregularity has generally been ascribed 85 to the inability to secure cotton from the same localities, it being well understood that cotton from different parts of the country produces mantles of quite different degrees of efficiency. The new process by more thoroughly eliminating the impurities brings all the mantles 90 up to nearly a uniform standard. The particular value of performing the bleaching operation after the knitting of the material is believed to lie chiefly in the better elimination 95 of the impurities introduced by the knitting operation and in the greater facility of handling, and consequently greater efficiency of bleaching operations upon a loosely-knitted tube as compared with loose skeins of thread. Furthermore, the crude cotton retaining its oil 100 can be knitted more rapidly by reason of the reduced friction between the threads and the needles and for the same reason takes up less or none of the metal of the needles. The greater facility of knitting an oily thread has 105 been demonstrated by experience, it having been found necessary sometimes to paraffin the thread in order to make it slip easily over the needles, (paraffin having to be subsequently extracted before impregnating it with incandescent material.) 110

The accompanying drawings illustrate a process embodying the invention, Figure 1 representing a tube knitted of unbleached cotton, Fig. 2 the same tube bleached, and Fig. 3 the bleached tube impregnated and ready for the usual burning.

Though I have described with great particularity of detail a certain specific process embodying the invention, yet it is not to be understood that the invention is limited to the specific process described. Various modifications thereof may be made by those skilled in the art without departure from the invention.

What I claim is—

- 15 1. The herein-described process of producing textile fabric for incandescent mantles, which consists in forming the same from raw threads containing impurities detrimental to the production of perfect impregnation, but 20 beneficial to the formation of the fabric, then removing the impurities by subjecting the fabric to a suitable reagent, and removing the reagent together with the impurities, and then impregnating with incandescing material.
- 20 2. The herein-described process of producing textile fabric for incandescent mantles,

which consists in forming the same from raw threads containing impurities detrimental to the production of perfect impregnation, but beneficial to the formation of the fabric, then 30 removing the impurities by subjecting the fabric to a suitable bleaching reagent, and removing the bleaching reagent together with the impurities, and then impregnating with incandescing material.

3. The herein-described process of producing textile fabric for incandescent mantles, which consists in forming the same from threads containing impurities detrimental to the production of perfect impregnation, but 40 beneficial to the formation of the fabric, then removing the impurities by subjecting the fabric to a suitable reagent, and removing the reagent together with the impurities, and then 45 impregnating with incandescing material.

In witness whereof I have hereunto signed my name in the presence of two subscribing witnesses.

OSCAR WIEDERHOLD.

Witnesses:

DOMINGO A. USINA,  
FRED WHITE.